

# United States Patent [19]

Sasaki et al.

[11] Patent Number: 4,997,752

[45] Date of Patent: Mar. 5, 1991

[54] **LIGHT-SENSITIVE SILVER HALIDE PHOTOGRAPHIC MATERIAL**

[75] Inventors: **Masao Sasaki, Hadano; Kaoru Onodera, Sagamihara, all of Japan**

[73] Assignee: **Konica Corporation, Tokyo, Japan**

[21] Appl. No.: **480,360**

[22] Filed: **Feb. 15, 1990**

**Related U.S. Application Data**

[63] Continuation of Ser. No. 186,941, Apr. 27, 1988, abandoned.

[30] **Foreign Application Priority Data**

Apr. 28, 1987 [JP] Japan ..... 62-105783

[51] Int. Cl.<sup>5</sup> ..... G03C 1/34; G03C 1/37

[52] U.S. Cl. ..... 430/611; 430/567;  
430/607; 430/613

[58] **Field of Search** ..... 430/567, 607, 611, 613,  
430/489, 490

[56] **References Cited**

**U.S. PATENT DOCUMENTS**

4,224,403 9/1980 Toda et al. ..... 430/537  
4,452,882 6/1984 Akimura et al. ..... 430/568

*Primary Examiner*—Hoa Van Le

*Attorney, Agent, or Firm*—Finnegan, Henderson,  
Farabow, Garrett, and Dunner

[57] **ABSTRACT**

A silver halide photographic light-sensitive material prevented from rottenness or decomposition by bacteria or mold without degradation of photographic properties such as sensitivity and fog. The silver halide photo-

graphic light-sensitive material has a photographic constituent layer containing at least one silver halide emulsion layer, and the silver halide grains contained in the emulsion layer comprises not less than 90 mole % of silver chloride. The photographic constituent layer contains at least one organic compound capable of forming a compound having a solubility product  $K_{sp}$  of not more than  $1 \times 10^{-11}$  with a silver ion, and at least one compound selected from the group of the compounds having the following Formula I, II, III or IV:



12 Claims, No Drawings

## LIGHT-SENSITIVE SILVER HALIDE PHOTOGRAPHIC MATERIAL

This application is a continuation of application No. 5 07/186,941 filed Apr. 27, 1988, now abandoned.

### FIELD OF THE INVENTION

The present invention relates to a light-sensitive silver halide photographic material which is so improved as to be restrained from the increase in fog as well as from the decline of its photographic speed even in its rapid processing, and is prevented satisfactorily from the rottenness or decomposition due to bacteria or mold even in its manufacture. 10

### BACKGROUND OF THE INVENTION

In recent years, there has been a growing demand for light-sensitive silver halide photographic materials capable of being rapidly processed to form high-quality 20 images.

The processing of light-sensitive silver halide photographic materials is usually performed continuously in the automatic processor that is installed in each photo-finishing laboratory, but for the improvement of photo-finishing service to customers, the processing of the accepted light-sensitive materials and return of photo-finished prints therefrom to customers within the day the light-sensitive materials were accepted has been required, and further, in nowadays, even quicker return 30 of them in the order of several hours to customers has now been required. Also from the standpoint that to shorten the processing time is to improve the productivity, enabling the reduction in cost, the development of rapid processing is urgently needed.

To accomplish the rapid processing, an approach thereto is made from both aspects of light-sensitive materials and processing solutions. As for color development, attempts have been made to use a high temperature, a high pH and a high color developing agent 40 concentration, and further the addition of additives such as a development accelerator and the like is also known. Examples of the development accelerator include the 1-phenyl-3-pyrazolidone as described in British Patent No. 811,185, the N-methyl-p-aminophenol as 45 described in U.S. Pat. No. 2,417,514, the N,N,N',N'-tetramethyl-p-phenylenediamine as described in Japanese Patent Publication Open to Public Inspection (hereinafter referred to as Japanese Patent O.P.I. Publication) No. 15554/1975, and the like. However, these methods are unable to accomplish any sufficient processing rapidity and liable to deteriorate light-sensitive materials' characteristics in such a way as increasing their fog.

On the other hand, it is well-known that the configuration, size and composition of the silver halide grain of 55 a silver halide emulsion to be used in a light-sensitive material largely affect the developing speed, and particularly the silver halide composition is significant—a significantly high developing speed is obtained particularly when a high chloride-containing silver halide is 60 used.

A light-sensitive material is produced generally through the preparation of its emulsion of a silver halide dispersed in an aqueous gelatin solution in the manufacturing process. The aqueous gelatin solution is known to 65 be decomposed or rotten by being subjected to the action of bacteria, mold or the like. For example, in the manufacture of a photographic material, an aqueous

gelatin solution containing photographic raw component materials, if allowed to stand in the gel or sol condition for a long period of time, becomes rotten or decomposed, leading to lowering its viscosity when used as a coating liquid, deteriorating the physical strength of the coated layer and bringing a coating trouble (e.g., comets) which is considered due to the decomposed product. These drawbacks have become serious problems in the rapid coating particularly for the mass production in recent years.

For the purpose of restraining such the rottenness or decomposition by bacteria, mold, etc., in a gelatin solution, various fungicides have been disclosed such as those in Japanese Patent O.P.I. Publication Nos. 27424/1979, 157244/1982, 84237/1984, 226344/1984, 263938/1985, 233743/1986, and the like.

We further investigated the problem by the application of various fungicides disclosed in the above publications to a silver halide light-sensitive material comprising a high silver chloride-content silver halide. As a result, it has become apparent that, as compared to silver chlorobromide-type conventional ones, the light-sensitive material is significant in the fog density increase as well as in the desensitization, and in addition, when processed continually over a long period, tends to show a significant desensitization and fog increase considered due to the fungicide dissolved out into its processing solution.

As a result of our various investigations for solving the above problem, it has now been found that by adding a certain restraining compound further to the above fungicide-added system, the fog density can be restrained and the sensitivity decline can be lessened without adversely affecting the processing rapidity, fungicidal effect, and the like, and thus the present invention has been completed.

### SUMMARY OF THE INVENTION

It is therefore an object of the present invention to provide a light-sensitive silver halide photographic material which is so improved as to be restrained from the increase in fog as well as from the decline of its sensitivity even in its rapid processing, and prevented satisfactorily from the rottenness or decomposition due to bacteria or mold even in its manufacture.

The above object of the present invention is accomplished by a light-sensitive silver halide photographic material comprising a support having thereon a photographic constituent layer including at least one silver halide emulsion layer, in which said silver halide emulsion layer contains silver halide grains whose silver chloride content is not less than 90 mole % and said photographic constituent layer contains at least one first compound selected from the group of organic compounds capable of forming a compound having a solubility product ( $K_{sp}$ ) of not more than  $1 \times 10^{-11}$  with a silver ion and at least one second compound selected from the group of compounds having the following Formulas I, II, III and IV.

Formula I





In Formulas I through IV, R<sub>1</sub> is a hydrogen atom, an alkyl or aryl group; R<sub>2</sub> is a hydrogen atom, a halogen atom, an alkyl, aryl, nitro, carboxy, sulfo, sulfamoyl, hydroxy, alkoxy or thiazolyl group; Z<sub>1</sub> is a group of non-metal atoms necessary to form a thiazoline ring; R<sub>3</sub> and R<sub>4</sub> each is an alkyl, aryl, —COR, or



group, wherein R, R' and R'' each is an alkyl or aryl group, provided that the R<sub>3</sub> and R<sub>4</sub> are allowed to form a ring together with the nitrogen atom; R<sub>5</sub>, R<sub>6</sub> and R<sub>7</sub> each is a halogen atom or an alkyl group; R<sub>8</sub> and R<sub>9</sub> each is a hydrogen atom, an alkyl, aryl or nitrogen-containing heterocyclic group; R<sub>10</sub> is a hydrogen atom, an alkyl, cycloalkyl, alkenyl, aryl, heterocyclic, alkylaminocarbonyl, arylaminocarbonyl, alkylaminosulfonyl or arylaminosulfonyl group; R<sub>11</sub> and R<sub>12</sub> each is a hydrogen atom, a halogen atom, an alkyl, cycloalkyl, aryl, cyano, alkylthio, arylthio, alkylsulfonyl, alkylsulfonyloxy or heterocyclic group, provided that the R<sub>11</sub> and R<sub>12</sub> are allowed to form a ring together.

In this invention, at least one layer of silver halide emulsion layers contains silver halide grains whose silver chloride content is not less than 90 mole %.

The silver chloride content of the silver halide grains of this invention is not less than 90 mole %, preferably not less than 95 mole %, and most preferably not less than 99 mole %. And it is desirable that the silver bromide content is not more than 5 mole % and the silver iodide content is not more than 0.5 mole %.

The silver halide grains of this invention may be used alone or in a mixture with other silver halide grains different in the composition, and may also be used in a mixture with silver halide grains whose silver chloride content is less than 10 mole %.

In the silver halide emulsion layer containing silver halide grains whose silver chloride content is not less than 90 mole %, the proportion of the silver halide grains containing not less than 90 mole % silver chloride to the whole silver halide grains contained in the emulsion layer is not less than 60% by weight, and preferably not less than 80% by weight.

The composition of the silver halide grain of this invention is allowed to be of either a homogeneous structure from the inside through the outside or a heterogeneous structure with the inside and outside different in the composition. Where the inside and outside of the

grain differ in the composition, the composition may vary either continuously or discontinuously.

The grain size range of the silver halide grains of this invention, although not particularly restricted, when taking into account the processing rapidity and other photographic characteristics such as the sensitivity, is preferably from 0.2 to 1.6  $\mu\text{m}$ , and more preferably from 0.25 to 1.2  $\mu\text{m}$ . The above grain size can be measured by any one of various measuring methods generally known to those skilled in the art. Typical methods are described in Loveland 'Analytical Methods for Grain Sizes', A.S.T.M. Symposium on Light Microscopy, pp. 94-122, 1955, and Mees and James 'Theory of the Photographic Process' 3rd. ed., Sec. 2, Macmillan, 1966.

The grain size may be measured by using either a projection area or a diameter's approximate value of the grain. If the silver halide grains are of a substantially uniform configuration, the grain size distribution thereof can be fairly precisely expressed in terms of the diameter or projection area.

The silver halide grains of this invention may be either polydisperse or monodisperse, but are preferably monodisperse silver halide grains which, in the silver halide grain size distribution thereof, have a coefficient of variation of not more than 0.22, and more preferably not more than 0.15, wherein the coefficient of variation is a coefficient representing the width of the grain size distribution, and defined by the following formula:

$$\text{Coefficient of variation } (S/r) = \frac{\text{Standard deviation of grain size distribution}}{\text{Average grain size}}$$

$$\text{Standard deviation of grain size distribution } (S) = \sqrt{\frac{\sum (r - r_i)^2 n_i}{\sum n_i}}$$

$$\text{Average grain size } (r) = \frac{\sum n_i r_i}{\sum n_i}$$

wherein r<sub>i</sub> represents each individual grain size, and n<sub>i</sub> is the number of grains. The term 'grain size' used herein, in the case of a spherical silver halide grain, means the diameter thereof and, in the case of a cubic or non-spherical grain, means the diameter of a circular image corresponding in the area to the projection image thereof.

The silver halide grain to be used in this invention can be of any arbitrary configuration. A preferred example of the configuration is a cube having a crystal {100} face. Also the silver halide grain may be prepared to be in the octahedral, tetrahedral or dodecahedral form in accordance with those methods as described in U.S. Pat. Nos. 4,183,756, 4,225,666, Japanese Patent O.P.I. Publication No. 26589/1980, Japanese Patent Examined Publication No. 42737/1980, and the like, and J. Photogr. Sci., 21, 39 (1973).

The silver halide grain to be used in this invention, by the addition of metal ions thereto in the course of being formed and/or grown by using a cadmium salt, zinc salt, lead salt, thallium salt, iridium salt or its complex salt, rhodium salt or its complex salt, or iron salt or its complex salt, can contain such metal ions in the inside and/or on the surface thereof and, by being allowed to stand in an appropriate reductive atmosphere, may be provided in the inside and/or on the surface thereof with a reduction sensitization nucleus.

The silver halide grain to be used in the emulsion of this invention is preferably a grain wherein a latent image is formed mainly on the surface thereof.

The emulsion of this invention may be chemically sensitized in usual manner. That is, the sensitization can be carried out by using alone or in combination the sulfur sensitization method, which uses active gelatin or a compound containing sulfur that is capable of reacting with silver ions; the selenium sensitization method, which uses a selenium compound; the reduction sensitization method, which uses a reductive material; the noble metal sensitization method, which uses a compound of gold or of other noble metal; and the like.

In this invention, as the chemical sensitizer, for example, chalcogen sensitizers may be used, and of these the sulfur sensitizer and selenium sensitizer are preferred. Examples of the sulfur sensitizer include, e.g., thiosulfates, allylthiocarbazine, thiourea, allylisothiocyanates, cystine, p-toluenthosulfonates, and rhodanine. And those sulfur sensitizers as described in U.S. Pat. Nos. 20 1,574,944, 2,410,689, 2,278,947, 2,728,668, 3,501,313, and 3,656,955, West German OLS Patent No. 1,422,869, and Japanese Patent O.P.I. Publication Nos. 24937/1981 and 45016/1980 may also be used. Adding amount of such the sulfur sensitizer varies in a fairly 25 wide range according to various conditions such as the pH, temperature, silver halide grain size and the like, but, as a standard, is preferably from  $10^{-7}$  mole to  $10^{-1}$  mole per mole of silver halide.

As the selenium sensitizer, aliphatic isoselenocyanates such as allylisoselenocyanates; selenothiourea; selenoketones; selenoamides; selenocarboxylic acid salts and esters; selenophosphates; and selenides such as diethyl selenide, diethyl diselenide, etc., may be used. Particular examples of these sensitizers are described in 35 U.S. Pat. Nos. 1,574,944, 1,602,592 and 1,623,499.

Further, a reduction sensitizer may be combinedly used. Examples of the reduction sensitizer include stannous chloride, thiourea dioxide, hydrazine, polyamine, and the like.

Further, non-gold noble metal compounds such as palladium compounds may also be used in combination.

The silver halide grain of this invention is desirable to contain a gold compound. The gold compound suitably usable in this invention may be either one having an oxidation number of +1 or one having an oxidation number of +3, and thus various gold compounds are allowed to be used, typical examples of which include chloroaurates such as potassium chloroaurate; auric trichloride, potassium auric thiocyanate, potassium 50 iodoaurate, tetracyano auric acid, ammonium aurothiocyanate, pyridyltrichloro gold, gold sulfide, gold selenide, and the like.

Any of such gold compounds may be used either so as to sensitize the silver halide grain or in such a way as 55 substantially not to contribute to the sensitization.

The adding amount of these gold compounds differs according to various conditions, but, as a standard, is from  $10^{-8}$  mole to  $10^{-1}$  mole per mole of silver halide, and preferably from  $10^{-7}$  mole to  $10^{-2}$  mole.

The addition of these compounds may be made at any point of time during the formation of silver halide grains, during the course of physical ripening, during the chemical ripening or after completion of the chemical ripening.

The silver halide grains to be used in the emulsion layer other than the silver halide emulsion layer of this invention, although not particularly restricted, are pref-

erably ones containing the same silver halide grains whose silver chloride content is not less than 90 mole % as used in the silver halide emulsion layer of this invention.

The emulsion of this invention may be spectrally sensitized to any desired wavelength regions by using those dyes known as sensitizing dyes to those skilled in the art. Such sensitizing dyes may be used alone or in combination of two or more thereof. Any of those supersensitizers which are dyes which in themselves have no spectral sensitization effect or compounds which do substantially not absorb visible rays but strengthen the sensitization effect of these sensitizing dyes may also be incorporated along with these sensitizing dyes into the emulsion.

Where the silver halide emulsion of this invention is to be used as a blue-sensitive emulsion, the emulsion is desirable to be spectrally sensitized by a sensitizing dye having the following Formula A:



Formula A

wherein  $Z_{21}$  and  $Z_{22}$  each is a group of atoms necessary to form a benzoxazole nucleus, naphthoxazole nucleus, benzoselenazole nucleus, naphthoselenazole nucleus, benzothiazole nucleus, naphthothiazole nucleus, benzimidazole nucleus, naphthoimidazole nucleus, pyridine nucleus, or quinoline nucleus, provided that these heterocyclic nucleus include those each having a substituent.

The substituent to the heterocyclic nucleus formed by the  $Z_{21}$  or  $Z_{22}$  includes a halogen atom, cyano group, methyl group, ethyl group, methoxy group or ethoxy group.

$R_{21}$  and  $R_{22}$  each is an alkyl group, alkenyl group or 40 aryl group, but preferably an alkyl group, more preferably a carboxyl or sulfo group-substituted alkyl group, and most preferably a sulfoalkyl group having from 1 to 4 carbon atoms.  $R_{23}$  is one selected from the class consisting of a hydrogen atom, methyl group and ethyl group.  $X_1^-$  represents an anion. And  $1_1$  is an integer of 0 or 1.

The most useful dyes among those sensitizing dyes having Formula A are those sensitizing dyes having the following Formula A':



Formula A'

wherein  $Y_{21}$  and  $Y_{22}$  each is a group of atoms necessary to form a benzene ring or naphthalene ring, both being 60 substitutable. The benzene ring and naphthalene ring formed by the  $Y_{21}$  and  $Y_{22}$  include those each having a substituent, and the substituent is preferably a halogen atom, cyano group, methyl group, ethyl group, methoxy group or ethoxy group.

65 The above  $R_{21}$ ,  $R_{22}$ ,  $R_{23}$ ,  $X_1^-$  and  $1_1$  are as defined in the foregoing Formula A.

Where the silver halide emulsion is to be used as a green-sensitive emulsion, the emulsion is desirable to be

spectrally sensitized by using a sensitizing dye having the following Formula B:



wherein  $Z_{31}$  and  $Z_{32}$  each is a group of atoms necessary to form a benzene ring or a naphthalene ring which each is condensed with an oxazole. The formed heterocyclic nucleus is allowed to be substituted by one of various substituents. The substituent is preferably a halogen atom, aryl group, alkyl group or alkoxy group, more preferably a halogen atom, phenyl group or methoxy group, and most preferably a phenyl group.

According to a preferred embodiment of this invention, the  $Z_{31}$  and  $Z_{32}$  represent benzene rings condensed with oxazole rings, and at least one of these benzene rings is substituted at its fifth position by a phenyl group, or one benzene ring is substituted at its fifth position by a phenyl group and the other is substituted at its fifth position by a halogen atom.

$R_{31}$  and  $R_{32}$  each is an alkyl group, alkenyl group or aryl group, preferably an alkyl group, more preferably an alkyl group substituted by a carboxyl or sulfo group, and still more preferably a sulfoalkyl group having from 1 to 4 carbon atoms, and most preferably a sulfoethyl group.

$R_{33}$  is a hydrogen atom or alkyl group having from 1 to 3 carbon atoms, and preferably a hydrogen atom or ethyl group.

$X_2^-$  is an anion, e.g., a halogen ion such as, of chlorine, bromine or iodine, or another anion such as of



$CH_3SO_4$ ,  $C_2H_5SO_4$  or the like, and  $l_2$  is an integer of 1 or 0, provided that the  $l_2$  is 0 when the compound forms a intramolecular salt.

Where the silver halide emulsion of this invention is used as a red-sensitive emulsion, the emulsion is desirable to be spectrally sensitized by using a sensitizing dye having the following formula C or a sensitizing dye having the following Formula D:



10 wherein R is a hydrogen atom or alkyl group;  $R_{41}$  through  $R_{44}$  each is an alkyl group or aryl group;  $Z_{41}$ ,  $Z_{42}$ ,  $Z_{44}$  and  $Z_{45}$  each is a group of atoms necessary to form a benzene ring or naphthalene ring which each is condensed with a thiazole ring or selenazole ring;  $Z_{43}$  is a group of hydrocarbon atoms necessary to form a 6-member ring;  $l_3$  is an integer of 1 or 2; Z is a sulfur atom or selenium atom; and  $X_3^-$  is an anion.

In the above formulas, the alkyl group represented by the R is a methyl, ethyl or propyl group. The R is preferably a hydrogen atom, methyl or ethyl group, and more preferably a hydrogen atom or ethyl group.

The  $R_{41}$ ,  $R_{42}$ ,  $R_{43}$  and  $R_{44}$  each is a group selected from the class consisting of a substitutable straight-chain or branched-chain alkyl group (such as, e.g., methyl, ethyl, propyl, chloroethyl, hydroxyethyl, methoxyethyl, acetoxyethyl, carboxymethyl, carboxyethyl, ethoxycarbonylmethyl, sulfoethyl, sulfopropyl, sulfobutyl,  $\beta$ -hydroxy- $\gamma$ -sulfoethyl, sulfate propyl, allyl, benzyl or the like) and a substitutable aryl group (such as phenyl, carboxyphenyl, sulfophenyl or the like).

The heterocyclic ring formed by the  $Z_{41}$ ,  $Z_{42}$ ,  $Z_{44}$  or  $Z_{45}$  is allowed to have a substituent. The substituent is preferably a halogen atom, aryl, alkyl or alkoxy group, and more preferably a halogen atom (such as chlorine), phenyl or methoxy group.

The  $X_3^-$  is an anion such as of Cl, Br, I,



45  $CH_3SO_4$ ,  $C_2H_5SO_4$  or the like; and  $l_3$  is an integer of 1 or 2, provided that the  $l_3$  is 1 when the compound forms an intramolecular salt.

The adding amount of any of those sensitizing dyes having Formula A, B, C or D, although not particularly restricted, is within the range of preferably from about  $1 \times 10^{-7}$  to about  $1 \times 10^{-3}$  mole per mole of silver halide, and more preferably from  $5 \times 10^{-6}$  to  $5 \times 10^{-4}$  mole.

Also, in the light-sensitive silver halide photographic material of this invention, at least one layer of its photographic constituent layer including the light-sensitive layers comprising the silver halide emulsion layer containing the foregoing silver halide grains of this invention and other silver halide emulsion layer and the non-light-sensitive layers such as an intermediate layer, protective layer, filter layer, antihalation layer and the like, contains at least one first compound selected from the organic compounds capable of forming a compound having a solubility product (Ksp) of not more than  $1 \times 10^{-11}$  with a silver ion and at least one second compound selected from the compounds having Formulas I, II, III and IV.

The organic compound whose solubility product (K<sub>sp</sub>) with silver ions is not more than  $1 \times 10^{-11}$  will now be explained below:

For measurement and calculation of the above-mentioned solubility product (K<sub>sp</sub>) with silver ions, reference can be made to the 'Shin-Jikken Kagaku Koza' ('New Experimental Chemistry Course') Vol. 1, pp.233-250.

The organic compound having the foregoing solubility product with silver ions of not more than  $1 \times 10^{-11}$  (hereinafter referred to as the organic compound of this invention) is preferably a mercapto compound having the following Formula S.



Formula S

wherein Q is a group of atoms necessary to form a 5- or 6-member heterocyclic ring or a 5- or 6-member heterocyclic ring condensed with a benzene or naphthalene ring; and M is a hydrogen atom or a cation.

Those mercapto compounds having Formula S which are suitably usable as the organic compound of this invention will then be explained:

In Formula S, the Q is a group of atoms necessary to form a 5- or 6-member heterocyclic ring or a 5- or 6-member heterocyclic ring condensed with a benzene or naphthalene ring, wherein the heterocyclic ring to be formed by the Q is, for example, an imidazole ring, tetrazole ring, thiazole ring, oxazole ring, selenazole ring, benzimidazole ring, naphthimidazole ring, benzothiazole ring, naphthothiazole ring, benzoselenazole ring, naphthoselenazole ring, benzoxazole ring, or the like.

The cation represented by the M is of, for example, an alkali metal (such as sodium, potassium), ammonium group, or the like.

The mercapto compounds having Formula S include those preferred mercapto compounds having Formulas SA, SB, SC and SD.



Formula SA

wherein R<sub>A</sub> is a hydrogen atom, alkyl group, alkoxy group, aryl group, halogen atom, carboxyl group or a salt thereof, sulfo group or a salt thereof, or amino group; Z<sub>A</sub> is —NH—, —O— or —S—; and M is the same as the M defined in Formula S.



wherein Ar represents



R<sub>B</sub> is an alkyl group, alkoxy group, carboxyl group or a salt thereof, sulfo group or a salt thereof, hydroxyl group, amino group, acylamino group, carbamoyl group or sulfonamido group; n is an integer of from 0 to 2; and M is the same as the M defined in Formula S.

In Formulas SA and SB, the alkyl group represented by the R<sub>A</sub> or R<sub>B</sub> is, for example, a methyl group, ethyl group, butyl group or the like; the alkoxy group is, for example, a methoxy group, ethoxy group or the like; and the salt of the carboxyl and sulfo groups is, for example, a sodium salt, ammonium salt, or the like.

In Formula SA, the aryl group represented by the R<sub>A</sub> is, for example, a phenyl group, naphthyl group or the like; and the halogen atom is, for example, a chlorine atom, bromine atom or the like.

In Formula SB, the acylamino group represented by the R<sub>B</sub> is, for example, a methylcarbonylamino group, benzoylamino group or the like; the carbamoyl group is, for example, an ethylcarbamoyl group, phenylcarbamoyl group, or the like; and the sulfonamido group is, for example, a methylsulfonamido group, phenylsulfonamido group, or the like.

The above-mentioned alkyl, alkoxy, aryl, amino, acylamino, carbamoyl and sulfonamido groups further include those each having a substituent.



wherein Z<sub>C</sub> is



50 an oxygen atom or sulfur atom; R<sub>C</sub> is a hydrogen atom, alkyl group, aryl group, alkenyl group, cycloalkyl group, —SR<sub>C1</sub>,



—NHCOR<sub>C4</sub>, —NHSO<sub>2</sub>R<sub>C5</sub> or heterocyclic group, 60 wherein R<sub>C1</sub> is a hydrogen atom, alkyl group, alkenyl group, cycloalkyl group, aryl group, —COR<sub>C4</sub>, or —SO<sub>2</sub>R<sub>C5</sub>, R<sub>C2</sub> and R<sub>C3</sub> each is a hydrogen atom, alkyl group or aryl group, and R<sub>C4</sub> and R<sub>C5</sub> each is an alkyl group or aryl group; and M is the same as the M defined in Formula S.

The alkyl group represented by the R<sub>C</sub>, R<sub>C1</sub>, R<sub>C2</sub>, R<sub>C3</sub>, R<sub>C4</sub> and R<sub>C5</sub> of Formula SC is, e.g., a methyl group, benzyl group, ethyl group, propyl group or the

like; the aryl group is, e.g., a phenyl group, naphthyl group or the like.

The alkenyl group represented by the  $R_C$  or  $R_{C1}$  is, e.g., propenyl group or the like; the cycloalkyl group is, e.g., a cyclohexyl group or the like. And the heterocyclic group represented by the  $R_C$  is, e.g., a furyl group, pyridinyl group or the like.

The alkyl and aryl groups represented by the above  $R_C$ ,  $R_{C1}$ ,  $R_{C2}$ ,  $R_{C3}$ ,  $R_{C4}$  or  $R_{C5}$ , the alkenyl and cycloalkyl groups represented by the  $R_C$  or  $R_{C1}$ , and the heterocyclic groups represented by the  $R_C$  further include those each having a substituent.



Formula SD 15

wherein and  $R_D$  and  $M$  are the same as the  $R_C$  and the  $M$ , respectively, defined in Formula SC. Also,  $R_{D1}$  and  $R_{D2}$  are the same as the  $R_{C1}$  and  $R_{C2}$ , respectively, defined in Formula SC.

The following are examples of the compounds having Formula S, but this invention is not limited to and by 25 the examples.



SA-1



SA-2

30



SA-3



SA-4

35



SA-5



SA-6

40



SA-7

SA-8



SB-1



SB-2



SB-3



SB-4



SB-5



SB-6



Exemplified compound

 $R_C$  $M$ 

|      |                    |       |
|------|--------------------|-------|
| SC-1 | $-C_2H_5$          | $-H$  |
| SC-2 | $-CH_2-CH=CH_2$    | $-H$  |
| SC-3 | $-CH=CH-CH_2-CH_3$ | $-H$  |
| SC-4 | $-C_7H_{15}$       | $-H$  |
| SC-5 | $-C_9H_{19}$       | $-Na$ |

SC-6



SC-7

 $-C_4H_9(t)$  $-H$

-continued

|       |  |      |
|-------|--|------|
| SC-8  |  | -H   |
| SC-9  |  | -H   |
| SC-10 |  | -H   |
| SC-11 |  | -H   |
| SC-12 |  | -NH4 |
| SC-13 |  | -H   |
| SC-14 |  | -H   |
| SC-15 |  | -H   |
| SC-16 |  | -H   |
| SC-17 |  | -H   |
| SC-18 |  | -H   |
| SC-19 |  | -H   |
| SC-20 |  | -H   |



| Exemplified compound | R <sub>C</sub>                     | M  |
|----------------------|------------------------------------|----|
| SC-21                | -H                                 | -H |
| SC-22                | -C <sub>2</sub> H <sub>5</sub>     | -H |
| SC-23                | -C <sub>4</sub> H <sub>9</sub> (t) | -H |
| SC-24                | -C <sub>6</sub> H <sub>13</sub>    | -H |

|       |  |    |
|-------|--|----|
| SC-25 |  | -H |
|-------|--|----|



-continued

|       |            |    |
|-------|------------|----|
| SC-26 |            | —H |
| SC-27 |            | —H |
| SC-28 |            | —H |
| SC-29 |            | —H |
| SC-30 | —NH2       | —H |
| SC-31 | —CH2CH=CH2 | —H |
| SC-32 | —SH        | —H |
| SC-33 | —NHCO2H5   | —H |



| Exemplified compound | $\text{R}_{\text{C}}$ | $\text{R}_{\text{C}1}$ | $\text{M}$ |
|----------------------|-----------------------|------------------------|------------|
| SC-34                | —C2H5                 | —H                     | —H         |
| SC-35                | —CH3                  | —CH3                   | —H         |
| SC-36                | —CH3                  |                        | —H         |
| SC-37                | —NHCOCH3              | —CH3                   | —H         |
| SC-38                |                       |                        | —H         |
| SC-39                | —NHCOCH3              | —COCH3                 | —H         |
| SC-40                | —NHCOCH3              |                        | —H         |



| Exemplified compound | $\text{R}_{\text{D}}$ | $\text{R}_{\text{D}1}$ | $\text{R}_{\text{D}2}$ | $\text{M}$ |
|----------------------|-----------------------|------------------------|------------------------|------------|
| SD-1                 | —C2H5                 | —CH3                   | —CH3                   | —H         |
| SD-2                 |                       | —CH3                   | —CH3                   | —H         |

-continued



These compounds having Formula S include those compounds as described in, e.g., Japanese Patent Examined Publication No. 28496/1965, Japanese Patent O.P.I. Publication No. 89034/1975, J. Chem. Soc. 49, 1748 (1927) and 4237 (1952), J. Org. Chem. 39, 2469 (1965), U.S. Pat. No. 2,824,001, J. Chem. Soc. 1723 (1951), Japanese Patent O.P.I. Publication No. 111846/1981, British Patent No. 1,275,701, U.S. Pat. Nos. 3,266,897, 2,403,927, and the like, and these compounds may be synthesized according to those methods as described also in these publications.

Incorporation of the compound having Formula S according to this invention (hereinafter referred to as Compound S) into the photographic constituent layer of this invention may be carried out in the manner that the compound is dissolved into water or an organic solvent miscible arbitrarily with water (such as methanol, ethanol, etc.), and the solution is then added to the constituent layer. Compounds S may be used alone or in combination of two or more thereof or in combination with stabilizers or antifoggants other than Compounds S.

The addition of Compound S may be made at any point of time during the period up to the completion of 60 coating liquid preparation.

Compound S may be added to any photographic constituent layer, and preferably to the silver halide emulsion layer.

To the photographic constituent layer may be added 65 the whole of Compound S at a time, but preferably in several installments.

The adding amount of Compound S, although not restricted, is in the range of normally from  $1 \times 10^{-6}$

mole to  $1 \times 10^{-1}$  mole per mole of silver halide, and preferably from  $1 \times 10^{-5}$  mole to  $1 \times 10^{-2}$  mole.

In this invention, at least one of the photographic constituent layers contains at least one second compound selected from the compounds having Formulas I through IV.

In Formulas I through IV, the  $R_1$  is a hydrogen atom, alkyl group or aryl group; the  $R_2$  is a hydrogen atom, halogen atom, alkyl group, aryl group, nitro group, carboxy group, sulfo group, sulfamoyl group, hydroxy group, alkoxy group or thiazolyl group; the  $Z_1$  is a group of non-metal atoms necessary to form a thiazoline ring; the  $R_3$  and  $R_4$  each is an alkyl group, aryl group,  $-\text{COR}$  or



wherein  $R'$  and  $R''$  each is an alkyl or aryl group, provided that the  $R_3$  and  $R_4$  are allowed to form a ring together with the nitrogen atom; the  $R_5$ ,  $R_6$  and  $R_7$  each is a halogen atom or alkyl group; the  $R_8$  and  $R_9$  each is a hydrogen atom, alkyl group, aryl group or nitrogen-containing heterocyclic ring; the  $R_{10}$  is a hydrogen atom, alkyl group, cycloalkyl group, alkenyl group, aryl group, heterocyclic group, alkylaminocarbonyl group, arylaminocarbonyl group, alkylaminosulfonyl group or arylaminosulfonyl group; the  $R_{11}$  and  $R_{12}$  each is a hydrogen atom, halogen atom, alkyl group, cycloal-

13  
kyl group, aryl group, cyano group, alkylthio group, arylthio group, alkylsulfonyl group, alkylsulfonyloxy group or heterocyclic group, provided that the  $R_{11}$  and  $R_{12}$  are allowed to form a ring together.

These substitutable groups represented by the above  $R_1$  through  $R_{12}$  may have further substituents.

These compounds having Formulas I through IV are known compounds and include those compounds as described in Japanese Patent O.P.I. Publication Nos. 10 27424/1979, 157244/1982, 84237/1984, 226344/1984, 263938/1985, 233743/1986, and the like.

The following are examples representative of the compounds having Formulas I through IV, but the invention is not limited to and by the examples. 15

### Exemplified Compounds



20

-continued  
Exemplified Compounds



L-8



10



J 10



11



113



11-3



114



II-5



II-6

-continued  
Exemplified Compounds



**-continued**  
**Exemplified Compounds**



-continued  
Exemplified Compounds



These compounds having Formulas I through IV may be added to any photographic constituent layer, but preferably to the non-light-sensitive layers when taking into account photographic characteristics. Any of the above compounds should be added at the time of preparing the colloid solution or emulsion for the photographic constituent layers, whereby possible rottenness or decomposition of the emulsion can be prevented.

The preferred among these compounds having Formulas I through IV are the compounds having Formulas I, II and IV, and more preferred are the compounds having Formulas I and IV.

The adding amount of the compound to the photographic constituent layers is preferably from  $5 \times 10^{-7}$  to  $2 \times 10^{-3}$  mole/m<sup>2</sup>, and more preferably from  $5 \times 10^{-6}$  to  $5 \times 10^{-4}$  mole/m<sup>2</sup>. When incorporating the compound into the light-sensitive material of this invention, it is desirable that the compound be dissolved into a solvent such as water, methanol, ethanol, ethylene glycol, diethylene glycol, triethylene glycol, benzyl alcohol, ethanolamine, diethanolamine, trimethanolamine or the like to prepare a solution or an emulsified liquid thereof, which is then added to the photographic constituent layers.

The light-sensitive silver halide photographic material of this invention having the above construction can be, for example, a color positive or negative film or a color photographic paper, but the effect of this invention can be well exhibited particularly when it is applied to color photographic paper, which is provided directly for appreciation.

The light-sensitive silver halide photographic material of this invention to be used principally as photographic paper may be for either monochromatic or multi-color use. Where it is a silver halide photographic

material for multi-color use, the light-sensitive material, for subtractive color reproduction, normally has a construction comprising a support having thereon an arbitrary number of silver halide emulsion layers separately containing photographic magenta coupler, yellow coupler and cyan coupler and non-light-sensitive layers, which are coated in an arbitrary order, but the number of and the coating order of such layers may be discretionarily changed according to the priority characteristic or the purpose for which the light-sensitive material is used.

Where the light-sensitive silver halide photographic material of this invention is a multi-color light-sensitive material, its concrete construction is particularly desirable to be such that on its support be arranged a yellow dye image-forming layer, an intermediate layer, a magenta dye image-forming layer, an intermediate layer, a cyan dye image-forming layer, an intermediate layer and a protective layer in the described order from the support side.

Thus, dye forming couplers are used in the light-sensitive silver halide photographic material of this invention. These dye forming couplers are desirable to have in the molecule thereof a group called 'ballasting group' having not less than 8 carbon atoms for making the coupler nondiffusible.

As the yellow dye-forming coupler, acylacetanilide-type couplers may be suitably used. Out of these couplers, benzoylacetanilide-type and pivaloylacetanilide-type compounds are advantageous, which are preferably those compounds having the following Formula Y:



wherein R<sub>Y1</sub> is a halogen atom or alkoxy group; R<sub>Y2</sub> is a hydrogen atom, halogen atom or alkoxy group; R<sub>Y3</sub> is an acylamino group, alkoxy carbonyl group, alkylsulfamoyl group, arylsulfamoyl group, arylsulfonamido group, alkylureido group, arylureido group, succinimido group, alkoxy group or aryloxy group; and Z<sub>Y1</sub> is a group capable of being split off upon the reaction with the oxidation product of a color developing agent.

Examples of the yellow coupler usable in this invention are those as described in British Patent No. 1,077,874, Japanese Patent Examined Publication No. 40757/1970, Japanese Patent O.P.I. Publication Nos. 1031/1972, 26133/1972, 94432/1973, 87650/1975, 3631/1976, 115219/1977, 99433/1979, 133329/1979 and 30127/1981, U.S. Pat. Nos. 2,875,057, 3,253,924, 3,265,506, 3,408,194, 3,551,155, 3,551,156, 3,664,841, 3,725,072, 3,730,722, 3,891,445, 3,900,483, 3,929,484, 3,933,500, 3,973,968, 3,990,896, 4,012,259, 4,022,620, 4,029,508, 4,057,432, 4,106,942, 4,133,958, 4,269,936, 4,286,053, 4,304,845, 4,314,023, 4,336,327, 4,356,258, 4,386,155 and 4,401,752.

As the magenta dye-forming coupler, 5-pyrazolone-type couplers, pyrazolozazole-type couplers and the like may be suitably used, which are preferably those couplers having the following Formulas P and M.



wherein  $Ar_P$  is an aryl group;  $R_{P1}$  is a hydrogen atom or a substituent;  $R_{P2}$  is a substituent;  $Y$  is a hydrogen atom or a group capable of being split off upon the reaction with the oxidation product of a color developing agent;  $W$  is  $-\text{NH}-$ ,  $-\text{NHCO}-$  (wherein the N atom is bonded to the carbon atom of the pyrazolone nucleus) or  $-\text{NHCONH}-$ ; and  $m$  is an integer of 1 or 2.



wherein  $Z_M$  is a group of non-metal atoms necessary to form a nitrogen-containing heterocyclic ring, and the ring to be formed by the  $Z_M$  may have a substituent;  $X$  is a group capable of being split off upon the reaction with the oxidation product of a color developing agent;  $R_M$  is a hydrogen atom or a substituent.

The substituent represented by the  $R_M$  is, for example, a halogen atom, alkyl group, cycloalkyl group, alkenyl group, cycloalkenyl group, alkinyl group, aryl group, heterocyclic group, acyl group, sulfonyl group, sulfinyl group, phosphonyl group, carbamoyl group, sulfamoyl group, cyano group, spiro compound residue, bridged hydrocarbon compound residue, alkoxy group, aryloxy group, heterocyclic oxy group, siloxy group, acyloxy group, carbamoyloxy group, amino group, acylamino group, sulfonamido group, imido group, ureido group, sulfamoyl amino group, alkoxy carbonylaminog group, aryloxycarbonylaminog group, alkoxycarbonyl group, aryloxycarbonyl group, alkylthio group, arylthio group or heterocyclic thio group.

These are described in, e.g., U.S. Pat. Nos. 2,600,788, 3,061,432, 3,062,653, 3,127,269, 3,311,476, 3,152,896, 3,419,391, 3,519,429, 3,555,318, 3,684,514, 3,888,680, 3,907,571, 3,928,044, 3,928,044, 3,930,861, 3,930,866 and 3,933,500, Japanese Patent O.P.I. Publication Nos. 29639/1974, 111631/1974, 129538/1974, 13041/1975, 58922/1977, 62454/1980, 118034/1980, 38043/1981, 35858/1982 and 23855/1985, British Patent No. 1,247,493, Belgian Patent Nos. 769,116 and 792,525, West German Patent No. 2,156,111, Japanese Patent Examined Publication No. 60479/1971, Japanese Patent O.P.I. Publication Nos. 125732/1984, 228252/1984, 162548/1984, 171956/1984, 333552/1985 and 43659/1985, West German Patent No. 1,070,030, and U.S. Pat. No. 3,725,067.

As the cyan dye-forming coupler, phenol-type and naphthol-type cyan couplers may be used, of which those couplers having the following Formulas E and F are preferably used.



5  
10  
15

wherein  $R_{E1}$  is an aryl group, cycloalkyl group or a heterocyclic group;  $R_{E2}$  is an alkyl group or phenyl group;  $R_{E3}$  is a hydrogen atom, halogen atom, alkyl group or alkoxy group;  $Z_{E1}$  is a hydrogen atom or a group capable of being split off upon the reaction with the oxidation product of a color developing agent.

20  
25



wherein  $R_{F4}$  is an alkyl group such as methyl, ethyl, propyl, butyl, nonyl;  $R_{F5}$  is an alkyl group such as methyl, ethyl;  $R_{F6}$  is a hydrogen atom, halogen atom such as fluorine, chlorine, bromine or alkyl group such as methyl, ethyl; and  $Z_{F2}$  is a hydrogen atom or a group capable of being split off upon the reaction with the oxidation product of a color developing agent.

These cyan dye image-forming couplers are described in U.S. Pat. Nos. 2,306,410, 2,356,475, 2,362,598, 2,367,531, 2,369,929, 2,432,730, 2,474,293, 2,476,008, 2,498,466, 2,545,687, 2,728,660, 2,772,162, 2,895,826, 2,976,146, 3,002,836, 3,419,390, 3,446,622, 3,476,563, 3,737,316, 3,758,308 and 3,839,044, British Patent Nos. 478,991, 945,542, 1,084,480, 1,377,233, 1,388,024 and 1,543,040, and Japanese Patent O.P.I. Publication Nos. 37425/1972, 10135/1975, 25228/1975, 112038/1975, 117422/1975, 130441/1975, 6551/1976, 37647/1976, 52828/1976, 108841/1976, 109630/1978, 48237/1979, 66129/1979, 131931/1979, 32071/1980, 146050/1984, 31953/1984 and 117249/1985.

The dye-forming coupler to be applied to this invention may be used in each silver halide emulsion layer in the range of normally from  $1 \times 10^{-3}$  mole to 1 mole per mole of silver halide, and preferably from  $1 \times 10^{-2}$  mole to  $8 \times 10^{-1}$  mole per mole of silver halide.

As the binder (or protective colloid) to be used in the light-sensitive silver halide photographic material of this invention, gelatin is advantageously used, and in addition, gelatin derivatives, graft polymers obtained from gelatin and other high molecular materials, protein, sugar derivatives, cellulose derivatives, and hydrophilic colloids including synthetic hydrophilic high-molecular materials such as homo- or copolymers may also be used.

In the light-sensitive silver halide photographic material of this invention, additives such as a hardening agent, anti-color-stain agent, image stabilizer, ultraviolet absorbing agent, plasticizer, latex, surface active agent, matting agent, lubricant, antistatic agent, and the like, may be arbitrarily used.

The light-sensitive silver halide photographic material of this invention is capable of forming an image by

being processed according to a color developing procedure known to those skilled in the art.

The light-sensitive silver halide photographic material of this invention is imagewise exposed and then developed in a color developer solution containing a color developing agent. Useful examples of the color developing agent include N,N-diethyl-p-phenylenediamine hydrochloride, N-methyl-p-phenylenediamine hydrochloride, N,N-dimethyl-p-phenylenediamine hydrochloride, 2-amino-5-(N-ethyl-N-dodecylamino)-toluene, N-ethyl-N-β-methansulfonamidoethyl-3-methyl-4-aminoaniline sulfate, N-ethyl-N-β-hydroxyethylaminoaniline sulfate, 4-amino-3-methyl-N,N-dietylaniline hydrochloride, N-ethyl-N-β-hydroxyethyl-3-methyl-4-aminoaniline sulfate, 4-amino-N-(β-methoxyethyl)-N-ethyl-3-methylaniline-p-toluene sulfonate, and the like.

These color developing agents may be used alone or in combination of two or more thereof. The color developing agent concentration of a color developer solution may be appropriately selected within the range of from 0.01 mole to 0.05 mole per liter of a color developer solution.

The color developer solution is desirable to contain a hydroxylamine-type compound as a preservative. Any hydroxylamine-type compounds may be used with no restriction, which include, e.g., hydroxylamine; N-monoalkylhydroxylamines such as N-methylhydroxylamine hydrochloride; N,N-dialkylhydroxylamines such as N,N-diethylhydroxylamine, those aminoalkylhydroxylamines as described in U.S. Pat. No. 3,287,125, those alkoxyhydroxylamines as described in U.S. Pat. No. 3,293,034, those sulfonhydroxylamines as described in U.S. Pat. No. 3,287,124; and heterocyclic N-hydroxylamines such as N-hydroxypiperidine. These may be used as they are or in the salt form. However, from the standpoint of cost, stability, water-solubility, availability or aptitude for use, hydroxylamine sulfate, hydroxylamine hydrochloride, N,N-diethylhydroxylamine, N,N-diethylhydroxylamine oxalate or the like is preferred. The concentration of the hydroxylamine-type compound to be used, although it depends upon the pH or temperature of a color developer solution, is preferred to be in the range of from 0.01 mole to 0.2 mole per liter of a color developer solution, and more preferably from 0.010 mole to 0.10 mole.

Further, the color developer solution is desirable to contain a sulfite such as sodium sulfite or potassium sulfite in an amount of preferably not more than  $2 \times 10^{-2}$  mole/liter, more preferably  $1 \times 10^{-2}$  mole/liter, and most preferably from  $5 \times 10^{-3}$  to  $1 \times 10^{-2}$  mole/liter.

To the color developer solution is further added an ordinary alkali agent appropriately selected from the class consisting of sodium hydroxide, potassium hydroxide, ammonium hydroxide, sodium carbonate, potassium carbonate, sodium sulfate, sodium metaborate, sodium tertiary phosphate and potassium tertiary phosphate. Also, in order to provide an alkali-buffering capability to the solution, disodium hydrogenphosphate, dipotassium hydrogenphosphate, sodium dihydrogenphosphate, potassium dihydrogenphosphate, potassium hydrogencarbonate, sodium hydrogen carbonate, or other salts may be used.

Into the color developer solution may be arbitrarily incorporated various other additives such as, e.g., benzyl alcohol, halogenated alkalies such as potassium bromide, calcium chloride, etc., development control

agents such as citrazic acid, defoaming agent, surface active agent, and organic solvent such as methanol, dimethylformamide, dimethylsulfoxide, etc.

However, the benzyl alcohol is not always necessary for the color developer solution of this invention, and is desirable not to be used from an environmental pollution point of view. The bromide ion concentration, in potassium bromide equivalent, should be 0.4 to 2.0 g per liter of the color developer solution, and preferably from 0.6 to 1.5 g.

The pH value of the color developer solution is normally not less than 7, and most generally from about 10 to about 13.

The color developer solution temperature is normally not less than 15° C., and generally in the range of from 20° C. to 50° C. For rapid processing, the developer solution is desirable to be used at not less than 30° C. The conventional developing time is from 3 to 4 minutes, but the color developing time according to this invention, which is intended for rapid processing, is in general in the range of preferably from 20 to 60 seconds, and more preferably from 30 to 50 seconds.

The light-sensitive material to be used in this invention is color-developed to form a dye image, and after that both the undeveloped silver halide and the developed silver must be removed by a bleach-fix bath.

The bleach-fix bath basically contains both bleaching agent and fixing agent.

The bleach-fix process in this invention is a process to oxidize the metal silver that has been produced by development into a silver halide and then to form a water-soluble complex as well as to color-form the un-color-developed portion of the color developing agent.

As the bleaching agent to be used in the bleach-fix bath, an organic acid's metal complex salt is preferred, in which a metal ion such as iron, cobalt or copper is coordinated in an organic acid such as aminocarboxylic acid, oxalic acid or citric acid. The most preferred organic acids for use in forming such organic acid's metal complex salts are polycarboxylic acids. These polycarboxylic acids or aminopolycarboxylic acids are allowed to be in the form of alkali metal salts, ammonium salts or water-soluble amine salts.

The bleaching agent is used in an amount of from 5 to 450 g/liter, and more preferably from 20 to 250 g/liter.

The bleach-fix bath, in addition to the above bleaching agent, contains a silver halide fixing agent and, if necessary, an sulfite as a preservative.

Also, as the bleach-fix bath, a special composition having bleach-fix bath may also be used which is such as a bleach-fix bath comprised of a composition wherein a small amount of a halide such as ammonium bromide is added in addition to an iron (III) ethylenediaminetetraacetate complex salt bleaching agent and the foregoing silver halide fixing agent; a bleach-fix bath comprising a large amount of a halide such as ammonium bromide; or a bleach-fix bath of a composition in combination of the iron (III) ethylenediaminetetraacetate complex salt bleaching agent with a large amount of a halide such as ammonium bromide. As the halide, hydrochloric acid, hydrobromic acid, lithium bromide, sodium bromide, potassium bromide, sodium iodide, potassium iodide, ammonium iodide or the like may also be used in addition to the above-mentioned ammonium bromide.

As the foregoing silver halide fixing agent to be contained in the bleach-fix bath, a compound to react with silver halide to form a water-soluble complex salt, which is usually used in fixing, may be used, typical

examples of which include thiosulfates such as, e.g., potassium thiosulfate, sodium thiosulfate, ammonium thiosulfate, etc., thiocyanates such as potassium thiocyanate, sodium thiocyanate, ammonium thiocyanate, etc., thiourea, thioether, and the like. These fixing agents are used in an amount of not less than 5 g/liter, or may be used in an amount to a dissolvable extent, but are generally used in the amount range of from 70 g to 250 g/liter.

The bleach-fix bath may contain various pH buffers such as boric acid, borax, sodium hydroxide, potassium hydroxide, sodium carbonate, potassium carbonate, sodium hydrogencarbonate, potassium hydrogencarbonate, acetic acid, sodium acetate, ammonium hydroxide, and the like. These may be used alone or in combination of two or more thereof. The bleach-fix bath may also contain various brightening agents or surface active agents, and may further contain arbitrarily preservatives such as hydrogensulfite addition products of hydroxylamine, hydrazine and aldehyde compounds organic chelating agents such as aminopolycarboxylic acids, stabilizers such as nitro alcohol, nitrates, etc., and organic solvents such as methanol, dimethylsulfonamide, dimethylsulfoxide, and the like.

The bleach-fix bath to be used in this invention may also contain any of those various bleaching accelerating agents as described in Japanese Patent O.P.I. Publication No. 280/1976, Japanese Patent Examined Publication Nos. 8506/1970 and 556/1971, Belgian Patent No. 770,910, Japanese Patent Examined Publication Nos. 8836/1970 and 9854/1978, and Japanese Patent O.P.I. Publication Nos. 71634/1979 and 42349/1974.

The bleach-fix bath is used at a pH of not less than 4.0, generally in the pH range of from 5.0 to 9.5, preferably from 6.0 to 8.5, and most preferably from 6.5 to 8.5. The 35 bleach-fix processing takes place at a temperature of not more than 80° C., or more than 3° C. lower, preferably more than 5° C. lower than the color developer solution's temperature, and is desirable to take place at a temperature of not more than 55° C. with its loss by 40 evaporation being restrained.

The bleach-fix processing time is within 90 seconds and preferably within 60 seconds.

The color photographic light-sensitive material, after being subjected to color development and bleach-fix 45 bath processing, needs to have the disused chemicals remaining thereinside removed therefrom by washing.

but instead of the washing, may be subjected to a washing-substitution stabilizing treatment like those as described in Japanese Patent O.P.I. Publication Nos. 14834/1983, 105145/1983, 134634/1983 and 18631/1983, and Japanese Patent Application Nos. 2709/1983 and 89288/1984.

In the case where the color developer, bleach-fix and stabilizer solutions are used for processing while being continuously replenished by appropriate replenishers, the replenishing ration of each replenisher is from 100 to 1000 ml per m<sup>2</sup> of a color light-sensitive material, and preferably from 150 to 500 ml.

### Example-1

Silver chlorobromide emulsions and a silver chloride emulsion as shown below were prepared in accordance with the double jet process.

| Emulsion No.          | grain size<br>( $\mu\text{m}$ ) | Silver chloride<br>content (mol %) |
|-----------------------|---------------------------------|------------------------------------|
| Em-A<br>(comparative) | 0.5                             | 20                                 |
| Em-B<br>(comparative) | 0.5                             | 50                                 |
| Em-C<br>(invention)   | 0.5                             | 90                                 |
| Em-D<br>(invention)   | 0.5                             | 95                                 |
| Em-E<br>(invention)   | 0.5                             | 100                                |
| Em-F<br>(invention)   | 0.8                             | 95                                 |

Each of the above Emulsions Em-A through -F was chemically sensitized by adding thereto chloroauric acid in an amount of  $5 \times 10^{-5}$  mole per mole of silver halide and sodium thiosulfate in an amount of 2 mg per mole of silver halide. Emulsion Em-F was spectrally sensitized by using the following Sensitizing Dye A-1 and was regarded as Blue-Sensitive Emulsion-1 to be used hereinafter. Emulsion Em-D was spectrally sensitized by using the following Sensitizing Dye A-2 and was regarded as Green-Sensitive Emulsion-1. And Emulsions Em-A through Em-E were spectrally sensitized by using the following Sensitizing Dye A-3, whereby Red-Sensitive Emulsions-1 through -5 were obtained.



### Sensitizing Dye A-2



-continued

## Sensitizing Dye A-3



15

On a polyethylene-coated paper support were coated the following Layer 1 and Layer 2, whereby monochromatic light-sensitive material Samples No. 1 through No. 22.

20

## Layer 1: Red-sensitive emulsion layer

The emulsion was coated so that its constituents' respective coating weights are as follows: the above Red-Sensitive Emulsions-1 through -5 each . . . 2.5 mg/dm<sup>2</sup> in silver equivalent, the following Cyan Coupler C-1 . . . 1 mg/dm<sup>2</sup>, Cyan Coupler C-2 . . . 3 mg/dm<sup>2</sup>, High-Boiling Organic Solvent S-1 . . . 2 mg/dm<sup>2</sup>, [S] Compound or its comparative compound given in the following Table-1 . . .  $1.5 \times 10^{-4}$  mole/mol of AgX, the following Water-Soluble Dye-1 . . . 0.1 mg/dm<sup>2</sup>, Water-Soluble Dye-2 . . . 0.05 mg/dm<sup>2</sup>, gelatin . . . 14 mg/dm<sup>2</sup>, and the following Hardener H-1 . . . 0.05 mg/dm<sup>2</sup>.

## Layer 2: Protective layer

The protective layer was coated so that its constituents' coating weights are: the compounds having Formulas I through IV given in Table-1 each . . .  $5 \times 10^{-7}$  mole/dm<sup>2</sup>, gelatin . . . 20 mg/dm<sup>2</sup> and Hardener H-1 . . . 1 mg/dm<sup>2</sup>.

35

## Cyan Coupler C-1



40

## Cyan Coupler C-2



45

## High-Boiling Organic Solvent S-1



## Water-Soluble Dye-1

15



## Water-Soluble Dye-2



## Hardener H-1



The above-prepared samples each in part was exposed through an optical wedge by using a sensitometer KS-7 (Konishiroku Photo Industry Co., Ltd.) and in part remained unexposed, and then both parts were processed in the following procedure steps:

|    | Processing Steps                                                   | Temperature        | Time       |
|----|--------------------------------------------------------------------|--------------------|------------|
| 50 | Color developing                                                   | 34.7 $\pm$ 0.3° C. | 50 seconds |
|    | Bleach fix                                                         | 34.7 $\pm$ 0.3° C. | 50 seconds |
|    | Stabilizing                                                        | 30 . . . 34° C.    | 90 seconds |
|    | Drying                                                             | 60 . . . 80° C.    | 60 seconds |
| 55 | Color Developer Solution:                                          |                    |            |
|    | Pure water                                                         |                    | 800 ml     |
|    | Ethylene glycol                                                    |                    | 10 ml      |
|    | N,N-diethylhydroxylamine                                           |                    | 10 g       |
|    | Potassium chloride                                                 |                    | 2 g        |
|    | Potassium sulfite                                                  |                    | 0.1 g      |
|    | N-ethyl-N-β-methansulfonamidoethyl-3-methyl-4-aminoaniline sulfate |                    | 5 g        |
|    | Sodium tetrapolyphosphate                                          |                    | 2 g        |
| 60 | Potassium carbonate                                                |                    | 30 g       |
|    | Brightening agent (4,4'-diaminostilbenedisulfone derivative)       |                    | 1 g        |
|    | Water to make 1 liter. Adjust the pH to 10.8.                      |                    |            |
|    | Bleach-Fix Bath:                                                   |                    |            |
|    | Ferric-ammonium ethylenediaminetetraacetate, dihydrated            |                    | 60 g       |
| 65 | Ethylenediaminetetraacetic acid                                    |                    | 3 g        |
|    | Ammonium thiosulfate (aqueous 70% solution)                        |                    | 100 ml     |
|    | Ammonium sulfite (aqueous 40% solution)                            |                    | 27.5 ml    |
|    | Adjust the pH to 7.1, and then add water                           |                    |            |

-continued

to make 1 liter.  
Stabilizer bath

5-Chloro-2-methyl-4-isothiazoline-3-one 1 g  
1-Hydroxyethylidene-1,1-disulfonic acid 2 g  
Water to make 1 liter. Use sulfuric acid or potassium hydroxide to adjust the pH to 7.0.

hydroxide to adjust the pH to 7.0.

The above exposed and unexposed samples were subjected to the following characteristics tests. Their 10 results are collectively given in Table-1.

(1) Sensitometry:

Each exposed sample, after being processed as in the above, was subjected to sensitometric measurement by using a densitometer PDA-65 (manufactured by Konishiroku Photo Industry Co., Ltd.) to thereby find its photographic speed and fog values. The photographic speed of each sample is shown in the table in a relative speed to the speed of Sample No. 5 regarded as 100. The fog value was found by processing each sample in the same manner except extending the color developing time alone to 90 seconds. 20

(2) Mold/Bacteria Resistance Test:

The evaluation method described in Japanese Patent O.P.I. Publication No. 226343/1984 was used as a method for evaluating the improvement effect of the compounds having Formulas I to IV according to this invention.

The test results of these compounds in the example are as given in the following table. 25

|        |  | Number of molds per ml |  |
|--------|--|------------------------|--|
| I-1    |  | 0                      |  |
| I-4    |  | 0                      |  |
| II-2   |  | 0                      |  |
| III-1  |  | 0                      |  |
| IV-1   |  | 0                      |  |
| IV-3   |  | 0                      |  |
| IV-8   |  | 0                      |  |
| None   |  | $2 \times 10^7$        |  |
| Phenol |  | $4 \times 10^7$        |  |

TABLE I

| Sample No. | Layer 1 |            | Layer 2       |                  | Relative speed | Fog  |
|------------|---------|------------|---------------|------------------|----------------|------|
|            | EM      | AgCl ratio | [S] Compound  | Compound I to IV |                |      |
| 1          | 1'      | 20         | —             | —                | 62             | 0.06 |
| 2          | 1'      | 20         | SA-7          | —                | 48             | 0.05 |
| 3          | 1'      | 20         | —             | IV-1             | 62             | 0.06 |
| 4          | 1'      | 20         | SA-7          | IV-1             | 46             | 0.06 |
| 5          | 5       | 100        | —             | —                | 100            | 0.08 |
| 6          | 5       | 100        | SA-7          | —                | 99             | 0.05 |
| 7          | 5       | 100        | —             | IV-1             | 92             | 0.09 |
| 8          | 5       | 100        | SA-7          | IV-1             | 100            | 0.05 |
| 9          | 4       | 95         | SA-7          | IV-1             | 101            | 0.05 |
| 10         | 3       | 90         | SA-7          | IV-1             | 100            | 0.05 |
| 11         | 2       | 50         | SA-7          | IV-1             | 69             | 0.06 |
| 12         | 5       | 100        | SB-1          | IV-1             | 99             | 0.05 |
| 13         | 5       | 100        | SC-30         | IV-1             | 100            | 0.05 |
| 14         | 5       | 100        | SC-39         | IV-1             | 99             | 0.05 |
| 15         | 5       | 100        | SD-5          | IV-1             | 101            | 0.05 |
| 16         | 5       | 100        | SD-5          | I-1              | 102            | 0.05 |
| 17         | 5       | 100        | SD-5          | I-4              | 100            | 0.05 |
| 18         | 5       | 100        | SD-5          | II-2             | 101            | 0.06 |
| 19         | 5       | 100        | SD-5          | III-1            | 99             | 0.05 |
| 20         | 5       | 100        | SD-5          | IV-3             | 101            | 0.05 |
| 21         | 5       | 100        | SD-5          | IV-8             | 100            | 0.05 |
| 22         | 5       | 100        | Comparative-1 | IV-8             | 85             | 0.07 |

Note: Comp.: Comparative. Inv.: Invention

The structural formula and the solubility product (Ksp) with silver ions of the compound Comparative-1

that was used for comparison with [S] Compound, and the solubility product (Ksp) with silver ions of each [S] Compound are as follows:

Comparative-1



|       |                                |
|-------|--------------------------------|
| SA-7  | $K_{sp} = 2.1 \times 10^{-14}$ |
| SB-1  | $K_{sp} = 1.0 \times 10^{-17}$ |
| SC-30 | $K_{sp} = 1.9 \times 10^{-12}$ |
| SC-39 | $K_{sp} = 5.2 \times 10^{-13}$ |
| SD-5  | $K_{sp} = 3.4 \times 10^{-16}$ |

As is apparent from the results given in Table-1, Samples 1 through 4 and 11, whose each Layer-1 uses a non-invention emulsion, show that their aptitude for the foregoing rapid processing is poor, thus having low photographic speeds.

On the other hand, as for Samples 5 through 8, whose each emulsion is for this invention, Sample 7, to which was added Compound IV-1, shows the deterioration of its photographic speed and increase in fog. In contrast, Sample 8, which is one prepared by adding a compound whose Ksp is within the range specified in this invention to Sample 7, shows being substantially free from the above deterioration of photographic speed and fog—this obviously shows a surprising effect by comparison with the fact that Samples 2 and 6 are lower in the photographic speed than Samples 1 and 5, respectively.

Further, by comparison between Samples 4, 11, 10, 9 and 8, it is apparent that where the silver chloride ratio is low, no sufficient photographic speed can be obtained in rapid processing.

Also, Sample 22, which used a compound whose Ksp is out of the range specified in this invention, shows that it is inadequate in respect of its photographic speed and fog.

From the above results and the mold/bacteria test

results it is apparent that the samples of this invention

alone show that they are restrained from the speed decline and fog even in rapid processing, and further prevented well from the rottenness or decomposition due to bacteria or mold.

Example-2

Using the Blue-Sensitive Emulsion-1, Green-Sensitive Emulsion-1 and Red-Sensitive Emulsion-5, which were prepared in Example-1, the following respective layers were coated on a polyethylene-coated paper support in the described order from the support side, whereby multi-color light-sensitive photographic materials Samples No. 23 through No. 26 were prepared.

Layer 1: Blue-sensitive emulsion layer

The layer was coated so that its constituents have the following coating weights: the yellow coupler as shown in Table 2 . . . 8 mg/dm<sup>2</sup>, Blue-Sensitive Emulsion-1 . . . 3 mg/dm<sup>2</sup> in silver equivalent, High-Boiling Organic Solvent S-2 . . . 3 mg/dm<sup>2</sup>, and gelatin . . . 16 mg/dm<sup>2</sup>.

Layer 2: Intermediate layer

The layer was coated so that the coating weight of Hydroquinone Derivative HQ-1 is 0.45 mg/dm<sup>2</sup> and of gelatin is 10 mg/dm<sup>2</sup>.

Layer 3: Green-sensitive emulsion layer

The layer was coated so that its constituents have the following coating weights: the magenta coupler given in Table-2 . . . in coating weight as shown in Table-2, Water-Soluble Dye-3 . . . 0.1 mg/dm<sup>2</sup>, Green-Sensitive Emulsion-1 . . . 3.5 mg/dm<sup>2</sup> in silver equivalent, High-Boiling Solvent S-1 . . . 4 mg/dm<sup>2</sup>, and gelatin . . . 16 mg/dm<sup>2</sup>.

Layer 4: Intermediate layer

The layer was coated so that its constituents have the following coating weights: Ultraviolet Absorbing Agent UV-1 . . . 3 mg/dm<sup>2</sup> and UV-2 . . . 3 mg/dm<sup>2</sup>,

High-Boiling Organic Solvent S-2 . . . 4 mg/dm<sup>2</sup>, Hydroquinone Derivative HQ-1 . . . 0.45 mg/dm<sup>2</sup>, and gelatin . . . 14 mg/dm<sup>2</sup>.

Layer 5: Red-sensitive emulsion layer

The layer was coated so that its constituents have the following coating weights: Cyan Coupler C-1 . . . 1 mg/dm<sup>2</sup> and C-2 . . . 3 mg/dm<sup>2</sup>, High-Boiling Organic Solvent S-1 . . . 2 mg/dm<sup>2</sup>, Red-Sensitive Emulsion-5 . . . 2.5 mg/dm<sup>2</sup> in silver equivalent, Water-Soluble Dye-1 . . . 0.1 mg/dm<sup>2</sup>, Water-Soluble Dye-2 . . . 0.05 mg/dm<sup>2</sup>, SB-5 as [S] compound . . .  $1.5 \times 10^{-4}$  mole per mole of AgX and gelatin . . . 14 mg/dm<sup>2</sup>.

Layer 6: Intermediate layer

The layer was coated so that its constituents have the following coating weights: Ultraviolet Absorbing Agent UV-1 . . . 2 mg/dm<sup>2</sup> and UV-2 . . . 2 mg/dm<sup>2</sup>, High-Boiling Organic Solvent S-2 . . . 2 mg/dm<sup>2</sup>, and gelatin . . . 6 mg/dm<sup>2</sup>.

Layer 7: Protective layer

The layer was coated so that the coating weight of Fungicide IV-2 is  $5 \times 10^{-7}$  mole/dm<sup>2</sup> and of gelatin is 9 mg/dm<sup>2</sup>.

Further, Sample 27 was obtained in the same manner as in Sample 23 except that no [S] Compound was used in its Layer 5.

The above-obtained Samples 23 through 26 each was processed in the same manner as in Example-1 and then evaluated likewise, provided, however, that the photographic speeds of these samples are given in relative values to the speed of Sample 23 regarded as 100, and the relative speed and fog were found with respect to the blue-sensitive layer (B), green-sensitive layer (G) and red-sensitive layer (R). The obtained results are collectively shown in Table 2.

Y-1



Y-2



-continued

Y-3



M-1



M-2



M-3



M-4



C-3



39

4,997,752

40

-continued



### Hydroquinone Derivative HQ-1



### Water-Soluble Dye-3



TABLE 2

| Sample No. | Layer 1   |           | Layer                           |            | Layer 5 |     | Relative speed |      |      | Fog  |  |  |
|------------|-----------|-----------|---------------------------------|------------|---------|-----|----------------|------|------|------|--|--|
|            | Y Coupler | M Coupler | Coated Wt (mg/dm <sup>2</sup> ) | C Coupler  | B       | G   | R              | B    | G    | R    |  |  |
| 23         | Y-1       | M-1       | 3.5                             | C-1<br>C-2 | 100     | 100 | 100            | 0.05 | 0.05 | 0.05 |  |  |
| 24         | Y-2       | M-2       | 2.0                             | C-1        | 97      | 95  | 100            | 0.05 | 0.05 | 0.05 |  |  |

TABLE 2-continued

| Sample No.    | Y Coupler | Layer     |                                 | Layer 5           |     |     | Relative speed |      |      | Fog  |  |  |
|---------------|-----------|-----------|---------------------------------|-------------------|-----|-----|----------------|------|------|------|--|--|
|               |           | M Coupler | Coated Wt (mg/dm <sup>2</sup> ) | C Coupler         | B   | G   | R              | B    | G    | R    |  |  |
| 25            | Y-1       | M-3       | 2.0                             | C-3<br>C-4<br>C-3 | 100 | 98  | 100            | 0.05 | 0.05 | 0.05 |  |  |
| 26            | Y-3       | M-4       | 3.5                             | C-5               | 97  | 100 | 101            | 0.05 | 0.05 | 0.05 |  |  |
| 27<br>(Comp.) | Y-1       | M-1       | 3.5                             | C-1<br>C-2        | 100 | 100 | 92             | 0.05 | 0.06 | 0.09 |  |  |

As is apparent from the results shown in Table-2, the effect of this invention can be obtained likewise even in the multilayer-coated samples wherein couplers are variously changed.

What is claimed is:

1. A silver halide photographic light-sensitive material comprising a support having thereon a photographic constituent layer including at least one silver halide emulsion layer, wherein said silver halide emulsion layer contains silver halide grains of which silver chloride is present in an amount not less than 90 mole %, and said photographic constituent layer contains at least one first compound in an amount of  $1 \times 10^{-6}$  to  $1 \times 10^{-1}$  mole per mole of the silver halide contained in said emulsion layer selected from organic compounds capable of forming a compound having a solubility product  $K_{sp}$  of not more than  $1 \times 10^{-11}$  with a silver ion, and at least one second compound in an amount of  $5 \times 10^{-7}$  to  $2 \times 10^{-3}$  mole per square meter selected from the group consisting of the compounds having the following Formula I, II, III and IV:



Formula I

wherein R<sub>1</sub> represents a hydrogen atom, an alkyl group or an aryl group; R<sub>2</sub> represents a hydrogen atom, a halogen atom, an alkyl group, an aryl group, a nitro group, a carboxy group, a sulfo group, a sulfamoyl group, a hydroxy group, an alkoxy group or a thiazolyl group; Z<sub>1</sub> represents a group of non-metal atoms necessary to complete a thiazoline ring,



Formula II

wherein R<sub>3</sub> and R<sub>4</sub> each independently represents an alkyl group, an aryl group, —COR or



in which R, R' and R'' each independently represents an alkyl group or an aryl group, and R<sub>3</sub> and R<sub>4</sub> may be combined to form a ring together with the nitrogen atom; and R<sub>5</sub>, R<sub>6</sub> and R<sub>7</sub> each independently represents a halogen atom or an alkyl group,



Formula III

20 wherein R<sub>8</sub> and R<sub>9</sub> each independently represents a hydrogen atom, an alkyl group, an aryl group or a nitrogen-containing heterocyclic group,



Formula IV

25 wherein R<sub>10</sub> represents a hydrogen atom, an alkyl group, a cycloalkyl group, an alkenyl group, an aryl group, a heterocyclic group, an alkylaminocarbonyl group, an arylaminocarbonyl group, an alkylaminosulfonyl group or an arylaminosulfonyl group; R<sub>11</sub> and R<sub>12</sub> each independently represents a hydrogen atom, a halogen atom, an alkyl group, a cycloalkyl group, an aryl group, a cyano group, an alkylthio group, an arylthio group, an alkylsulfonyl group, an alkylsulfonyloxy group or a heterocyclic group, provided that the R<sub>11</sub> and R<sub>12</sub> may be combined with each other to form a ring.

30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930

five- or six-member heterocyclic ring condensed with a benzene ring or a naphthalene ring; and M represents a hydrogen atom or a cation.

7. The material of claim 6, wherein said first compound is selected from the compounds having the following Formula SA, SB, SC or SD:



Formula SA

wherein  $R_4$  represents a hydrogen atom, an alkyl group, an alkoxy group, an aryl group, a halogen atom, a carboxy group or a salt thereof, a sulfo group or a salt thereof or an amino group;  $Z_A$  represents  $-\text{NH}-$ ,  $-\text{O}-$  or  $-\text{S}-$ ; and M represents a hydrogen atom or a cation,



Formula SB

wherein Ar represents



in which  $R_B$  represents an alkyl group, an alkoxy group, a carboxy group or a salt thereof, a sulfo group or a salt thereof, a hydroxy group, an amino group, an acylamino group, a carbamoyl group or a sulfonamido group; n represents an integer of 0 to 2; and M is the same as the M defined in Formula SA,

45  
50

55



Formula SC

wherein  $Z_c$  represents a  $-\text{NRc}_1-$  group, an oxygen atom or a sulfur atom;  $R_c$  represents a hydrogen atom, an alkyl group, an aryl group, an alkenyl group, a cycloalkyl group, a  $\text{SRc}_1$  group, an  $-\text{NRC}_2\text{RC}_3$  group, an  $-\text{NHCORc}_4$  group, an  $-\text{NHSO}_2\text{RC}_5$  group or a heterocyclic group, wherein  $Rc_1$  represents a hydrogen atom, an alkyl group, an alkenyl group, a cycloalkyl group, an aryl group, a  $-\text{CORc}_4$  group or an  $-\text{SO}_2\text{RC}_5$  group,  $Rc_2$  and  $Rc_3$  each independently represents a hydrogen atom, an alkyl group or an aryl group,  $Rc_4$  and  $Rc_5$  each represents an alkyl group or an aryl group; and M is the same as the M defined in Formula SA,



Formula SD

wherein  $R_D$ , M,  $R_{D1}$  and  $R_{D2}$  and are the same as the  $R_c$ , M,  $Rc_1$  and  $Rc_2$ , respectively, defined in Formula SC.

8. The material of claim 1, wherein said first compound is contained in said silver halide emulsion layer.

9. The material of claim 1, wherein said second compound is contained in a non-light-sensitive layer included in said photographic constituent layer.

10. The material of claim 1, wherein said first compound is contained in said silver halide emulsion layer and said second compound is contained in a non-light-sensitive layer included in said photographic constituent layer.

11. The material of claim 1, wherein said compound having Formula S is contained in said photographic constituent layer in an amount of  $1 \times 10^{-5}$  to  $1 \times 10^{-2}$  mole per mole of the silver halide contained in said silver halide emulsion layer.

12. The material of claim 1, wherein said second compound is contained in said photographic constituent layer in an amount of  $5 \times 10^{-6}$  to  $5 \times 10^{-4}$  mole per square meter.

\* \* \* \* \*

60

65